

## [54] CARBOXYLIC ACID AMIDES

[72] Inventors: Hans Rudolf Biland, Gelterkinden; Max Duennenberger, Frenkendorf, both of Switzerland

[73] Assignee: Ciba Limited, Basel, Switzerland

[22] Filed: Dec. 4, 1969

[21] Appl. No.: 882,302

## [30] Foreign Application Priority Data

Dec. 13, 1968 Switzerland 18664/68

[52] U.S. Cl. 260/559 T, 252/402, 260/562 B,  
260/609 R, 260/45.9

[51] Int. Cl. C07c 103/22

[58] Field of Search 260/559 T; 252/402

## [56] References Cited

## OTHER PUBLICATIONS

Takahashi et al, Yakugaku Kenkyu, Vol. 36, 149- 162; (1965).

Primary Examiner—Henry R. Jiles

Assistant Examiner—S. D. Winters

Attorney—Harry Goldsmith, Joseph G. Kolodny and Mario A. Monaco

[57]

## ABSTRACT

The invention concerns new carboxylic acid amides of the formula



wherein M denotes a divalent bridge member of the series —S—, —S—A—S— and —S—CH<sub>2</sub>—CH<sub>2</sub>—(O—CH<sub>2</sub>—CH<sub>2</sub>)<sub>p</sub>—S—, A denotes an alkylene residue containing one to 18 carbon atoms, p denotes an integer from one to three, R<sub>1</sub> denotes an alkyl group and R<sub>2</sub> denotes alkyl or hydrogen.

These compounds are valuable antioxidants for polymers which are damaged by oxidative attacks.

4 Claims, No Drawings

## CARBOXYLIC ACID AMIDES

The subject of the invention is the new carboxylic acid amides of formula

(1)



wherein M denotes a divalent bridge member of the series —S—, —S—A—S— and —S—CH<sub>2</sub>—CH<sub>2</sub>—(O—CH<sub>2</sub>—CH<sub>2</sub>)<sub>p</sub>—S—, A denotes an alkylene residue containing 1 to 18 carbon atoms, p denotes an integer from one to three, R<sub>1</sub> denotes an alkyl group with one to eight carbon atoms and R<sub>2</sub> denotes hydrogen or an alkyl group with one to eight carbon atoms. Here the total number of carbon atoms for all "A" members normally does not amount to more than 36, preferably not more than 26.

In this formula, the alkylene residues A can be both straight-chain and branched in nature, but in any case represent divalent saturated residues. The substituents R<sub>1</sub> and R<sub>2</sub> can also be straight-chain or —preferably—branched in nature. Though both of the positions which are in each case possible for R<sub>1</sub> and R<sub>2</sub> can be considered, these residues are preferably in the o-position to the hydroxyl group.

Compounds of formula (1) of predominant practical interest are those which correspond to the formula

(2)



wherein M<sub>1</sub>' denotes a divalent bridge member —S—, —S—(CH<sub>2</sub>)<sub>q</sub>—S— or —S—CH<sub>2</sub>—CH<sub>2</sub>—O—CH<sub>2</sub>—CH<sub>2</sub>—S—, q denotes an integer from one to six, n denotes an integer from one to 12, R<sub>1</sub> denotes an alkyl group with one to eight carbon atoms, R<sub>2</sub> denotes hydrogen or an alkyl group with one to eight carbon atoms and R<sub>2</sub>' denotes hydrogen or an alkyl group containing one to four carbon atoms. In view of the fact that formula (2) lies within the framework of formula (1), it is obvious that R<sub>2</sub> and R<sub>2</sub>' cannot simultaneously be different from hydrogen.

Especially preferred types of compounds are those of the compounds of formula

(3)



wherein M<sub>1</sub> denotes a divalent bridge member —S— or —S—(CH<sub>2</sub>)<sub>q</sub>—S—, q denotes an integer from 1 to 6, n denotes an integer from 1 to 12, R<sub>1</sub> denotes an alkyl group with one to eight carbon atoms and R<sub>2</sub> denotes hydrogen or an alkyl group with one to eight carbon atoms (with the alkyl group for R<sub>1</sub> and R<sub>2</sub> in particular containing one to four carbon atoms), and furthermore compounds of formula

(4)



wherein M<sub>1</sub> denotes a divalent bridge member —S— or —S—(CH<sub>2</sub>)<sub>q</sub>—S—, q denotes an integer from one to six, m denotes an integer from one to four, and R<sub>3</sub> denotes a branched alkyl group containing one to four carbon atoms.

The compounds defined above can be manufactured analogously to procedures which are in themselves known. The compounds according to formula (1) — and analogously, those of the subordinate formulas — can appropriately be obtained by reacting about two mols of a compound of formula

75

(5)



with about one mol of a mercaptan of formula

(6)



15

in the form of its alkali salt, with R<sub>1</sub>, R<sub>2</sub>, A and M having the abovementioned significance and Hal representing a halogen atom.

Compounds of formula (2) are for example obtained entirely analogously by reacting about two mols of a compound of formula

(7)



with about 1 mol of a mercaptan of formula

(8)



in the form of its alkali salt, with R<sub>1</sub>, R<sub>2</sub>, R<sub>2</sub>', n and M<sub>1</sub>' having the abovementioned significance and Hal representing a halogen atom.

In the case where M<sub>1</sub> = —S—, compounds of formula (5) are for example condensed with sodium sulphide.

In the case where M<sub>1</sub> = —S—(CH<sub>2</sub>)<sub>q</sub>—S—, wherein q has the indicated significance, compounds of formula (5) are appropriately reacted with the alkali salts of dithiols formula



9

in a solvent which is inert towards the reagents (for example alcohols or hydrocarbons).

The alkali salts of the dithiols can be manufactured in the presence of a solvent by using the alkali metal, or through the use of the stoichiometric amount of an alkali alcoholate. The compounds of formula (5) required as starting substances are obtained by the reaction, which is in itself known, of acid ha-

60



lides, preferably acid chlorides, of formula



10

with p-aminophenols of formula

(11)



wherein A, Hal, R<sub>1</sub> and R<sub>2</sub> have the abovementioned significance. This reaction is carried out in the presence of a solvent which is inert towards the reagents, with the corresponding hydrogen halide acid being split off. The resulting hydrogen halide acid can be removed from the reaction mixture by sucking-off, or be bonded by adding a hydrogen halide acceptor, (for example a tertiary amine).

The compounds of formula (1) and of the subordinate formulas are suitable for stabilizing oxidation-sensitive organic materials against oxidation. For this purpose they can be used in a manner which is in itself known for the following substrates: homopolymers and copolymers of ethylenically unsaturated compounds such as vinyl chloride, vinylidene chloride, styrene, butadiene, isoprene, ethylene, propylene, acrylic and methacrylic acid derivatives, for example acrylic acid alkyl esters, acrylamides and acrylonitrile; polyamides, for example from  $\epsilon$ -caprolactam or from adipic acid and a diamine; polyesters such as polyterephthalic acid glycol ester; natural and synthetic rubbers; lubricating oils; petrol; vegetable and animal oils and fats; waxes; cellulose and cellulose derivatives such as cellulose esters.

The compounds defined above are of preferred importance as stabilizers against oxidative influences in the case of polymerization products of  $\alpha$ -olefines, that is to say in the case of homopolymers and copolymers of  $\alpha$ -olefines such as preferably ethylene or propylene, and also in the case of substrates which predominantly contain homopolymers or copolymers of  $\alpha$ -olefines.

For a good antioxidant effect, small amounts of compounds of formula (1), that is to say about 0.01 to two percent relative to the amount of the substrate to be protected, in general suffice. The antioxidants can for example be incorporated into the materials to be protected directly, that is to say by themselves, or together with other additives such as plasticizers, pigments, light protection agents or optical brighteners, and/or with the aid of solvents.

The antioxidative effect of the compounds of formula (1) also manifests itself in the light exposure test, in that these compounds are able to prevent or greatly to reduce oxidative processes induced by the action of light, for example the yellowing of polyethylene.

The symbols used in the formulas of the present description, such as  $R_1$ ,  $R_2$ ,  $m$  and  $n$ , throughout have the same significance which has been precisely circumscribed at least once. In the manufacturing instructions and examples which follow the parts denote parts by weight and the percentages denote percentages by weight unless otherwise stated.

### EXAMPLE 1

1.6 g of crystalline 61 percent strength sodium sulphide are dissolved in 100 ml of methanol. 7.425 g of the compound of formula



TABLE I

| Number: | R'                                 | R''                                | R'''            | A                                   | M | Melting<br>point,<br>°C. | Analysis of— |       |      |       |       |      |
|---------|------------------------------------|------------------------------------|-----------------|-------------------------------------|---|--------------------------|--------------|-------|------|-------|-------|------|
|         |                                    |                                    |                 |                                     |   |                          | Calculated   |       |      |       |       |      |
|         |                                    | C                                  | H               | N                                   |   | C                        | H            | N     |      |       |       |      |
| 14      | tert.C <sub>4</sub> H <sub>9</sub> | CH <sub>3</sub>                    | H               | —CH <sub>2</sub> —                  | S | 247-248                  | 66.07        | 7.68  | 5.93 | 65.78 | 8.00  | 5.75 |
| 15      | CH <sub>3</sub>                    | CH <sub>3</sub>                    | H               | —CH <sub>2</sub> —                  | S | 214-215                  | 61.83        | 6.23  | 7.21 | 61.60 | 6.30  | 7.29 |
| 16      | tert.C <sub>4</sub> H <sub>9</sub> | H                                  | H               | —CH <sub>2</sub> —                  | S | 217-218                  | 64.84        | 7.26  | 6.30 | 64.77 | 7.17  | 6.42 |
| 17      | tert.C <sub>4</sub> H <sub>9</sub> | H                                  | CH <sub>3</sub> | —CH <sub>2</sub> —                  | S | 270-271                  | 66.07        | 7.68  | 5.93 | 66.14 | 7.87  | 5.82 |
| 18      | tert.C <sub>4</sub> H <sub>9</sub> | tert.C <sub>4</sub> H <sub>9</sub> | H               | —(CH <sub>2</sub> ) <sub>2</sub> —  | S | 224-225                  | 63.82        | 8.96  | 4.79 | 69.57 | 9.08  | 4.86 |
| 19      | tert.C <sub>4</sub> H <sub>9</sub> | tert.C <sub>4</sub> H <sub>9</sub> | H               | —(CH <sub>2</sub> ) <sub>10</sub> — | S | 163-164                  | 74.21        | 10.46 | 3.46 | 74.50 | 10.44 | 3.40 |

dissolved in 10 ml of methanol are added thereto. The reaction solution is heated for 30 minutes to reflux temperature and is thereafter mixed with activated charcoal, filtered and concentrated to dryness.

5 Yield of crude product: 6.0 g (86.5 percent).

The product for analysis, recrystallized from methylene chloride/cyclohexane, of the compound of formula



15 shows the following data:

Melting point: 228° to 229° C.

Analysis: calculated: C 69.03 H 8.69 N 5.03

found: C 68.87 H 8.65 N 5.00

### The compound of formula



used as the starting material is manufactured as follows: 23.5 g of 2,6-di-tert. butyl-p-nitrosophenol are dissolved in 80 g of 5 N sodium hydroxide and diluted with 160 ml of water. A solution of 70 g of sodium hydrosulphite in 300 ml of water at about 50° C is added dropwise thereto while stirring. After completion of the addition of the sodium hydrosulphite the mixture is stirred for a further hour. The resulting crystal suspension is filtered off and washed with water until neutral. The moist filter cake of 2,6-di-tert.-butyl-p-aminophenol thus obtained is dissolved in 500 g of methylene chloride and separated from the aqueous phase. The methylene chloride phase is dried over sodium sulphate. After removing the drying agent, the mixture is concentrated to 300 g, 45 g of chloracetyl chloride are added dropwise at 20 to 30° C, and the whole stirred for 3 to 5 hours at reflux temperature until no further significant elimination of hydrogen chloride is detectable. The mixture is then finally stirred overnight at room temperature. Thereafter a few solid constituents are filtered off and the reaction solution is concentrated to dryness in vacuo. Yield of crude product: practically quantitative.

The products for analysis, recrystallized from cyclohexane, of formula (12) show the following data:

50 Melting point: 153° to 154°C

Analysis: calculated: C 64.53 H 8.12 N 4.70

found: C 64.38 H 8.17 N 4.77

The compounds quoted below are obtained in an analogous manner

The compounds of formula

(5a)



are obtained from the dried methylene chloride extracts.

The product for analysis, recrystallized from acetone/water, shows the following data:

Melting point: 200° to 201°C.

5 Analysis: calculated: C 66.19 H 8.50 N 4.54

found: C 65.91 H 8.53 N 4.46

The compounds quoted below are obtained in an analogous manner:



TABLE 3

| Number: | R'                                  | R''                                 | A                                   | M <sub>1</sub>                       | Melting point, °C. | Analysis of— |       |       |       |       |      |
|---------|-------------------------------------|-------------------------------------|-------------------------------------|--------------------------------------|--------------------|--------------|-------|-------|-------|-------|------|
|         |                                     |                                     |                                     |                                      |                    | Calculated   |       | Found |       |       |      |
|         |                                     |                                     |                                     |                                      |                    | C            | H     | N     | C     | H     | N    |
| 27      | tert. C <sub>4</sub> H <sub>9</sub> | CH <sub>3</sub>                     | —CH <sub>2</sub> —                  | —SCH <sub>2</sub> CH <sub>2</sub> S— | 237-238            | 63.12        | 7.57  | 5.26  | 63.04 | 7.58  | 5.08 |
| 28      | CH <sub>3</sub>                     | CH <sub>3</sub>                     | —CH <sub>2</sub> —                  | —SCH <sub>2</sub> CH <sub>2</sub> S— | 202-203            | 58.90        | 6.29  | 6.24  | 58.67 | 6.24  | 6.21 |
| 29      | iso-C <sub>3</sub> H <sub>7</sub>   | iso-C <sub>3</sub> H <sub>7</sub>   | —CH <sub>2</sub> —                  | —SCH <sub>2</sub> CH <sub>2</sub> S— | 182-183            | 64.25        | 7.91  | 5.00  | 63.94 | 7.71  | 4.86 |
| 30      | tert. C <sub>4</sub> H <sub>9</sub> | tert. C <sub>4</sub> H <sub>9</sub> | —CH <sub>2</sub> —                  | —S(CH <sub>2</sub> ) <sub>3</sub> S— | 194-195            | 66.63        | 8.63  | 4.44  | 66.30 | 8.56  | 4.59 |
| 31      | tert. C <sub>4</sub> H <sub>9</sub> | tert. C <sub>4</sub> H <sub>9</sub> | —CH <sub>2</sub> —                  | —S(CH <sub>2</sub> ) <sub>3</sub> S— | 218-219            | 67.04        | 8.75  | 4.34  | 66.81 | 9.01  | 4.16 |
| 32      | tert. C <sub>4</sub> H <sub>9</sub> | tert. C <sub>4</sub> H <sub>9</sub> | —CH <sub>2</sub> —                  | —S(CH <sub>2</sub> ) <sub>3</sub> S— | 188-190            | 67.81        | 8.99  | 4.16  | 67.52 | 9.21  | 3.93 |
| 33      | tert. C <sub>4</sub> H <sub>9</sub> | tert. C <sub>4</sub> H <sub>9</sub> | —(CH <sub>2</sub> ) <sub>10</sub> — | —SCH <sub>2</sub> CH <sub>2</sub> S— | 58-60              | 71.84        | 10.20 | 3.22  | 71.88 | 10.14 | 2.97 |

(34)



used as the starting material, having the significance given in Table 2 for R', R'', R''', A and Hal are obtained by reaction of the appropriate acid chloride with the appropriately substituted p-aminophenol.

The compound of formula

Melting point: 174° to 176°C.

Analysis: calculated: C 65.42 H 8.54 N 4.24

found: C 65.64 H 8.72 N 4.21

40

TABLE 2

| Number: | R'                                  | R''                                 | R'''            | A                                   | Melting point, °C. | Hal |    |   |
|---------|-------------------------------------|-------------------------------------|-----------------|-------------------------------------|--------------------|-----|----|---|
|         |                                     |                                     |                 |                                     |                    | Cl  | Br | I |
| 20      | tert. C <sub>4</sub> H <sub>9</sub> | CH <sub>3</sub>                     | H               | —CH <sub>2</sub> —                  | 185-186            | Cl  |    |   |
| 21      | CH <sub>3</sub>                     | CH <sub>3</sub>                     | H               | —CH <sub>2</sub> —                  | 163-164            | Cl  |    |   |
| 22      | tert. C <sub>4</sub> H <sub>9</sub> | H                                   | H               | —CH <sub>2</sub> —                  | 107-109            | Cl  |    |   |
| 23      | tert. C <sub>4</sub> H <sub>9</sub> | H                                   | CH <sub>3</sub> | —CH <sub>2</sub> —                  | 150-151            | Cl  |    |   |
| 24      | tert. C <sub>4</sub> H <sub>9</sub> | tert. C <sub>4</sub> H <sub>9</sub> | H               | —(CH <sub>2</sub> ) <sub>2</sub> —  | 171.5-172          | Cl  |    |   |
| 25      | tert. C <sub>4</sub> H <sub>9</sub> | tert. C <sub>4</sub> H <sub>9</sub> | H               | —(CH <sub>2</sub> ) <sub>10</sub> — | 109-111            | Br  |    |   |

### EXAMPLE 2

The mercaptide of 1,2-ethanediol is manufactured by introducing 580 mg of sodium into a solution of 1,2-ethanediol in 20 ml of absolute alcohol. 7.45 g of the compound of formula



dissolved in 70 ml of absolute ethanol are added to this solution. Thereafter the reaction solution is heated to reflux temperature for one hour and subsequently concentrated to dryness in vacuo, and the residue is taken up in methylene chloride and extracted by shaking with water. 4.0 g of crude product of the compound of formula



55 A mixture of 100 g of unstabilized polypropylene (Profax 6501, Hercules powder) and 0.2 g of a compound according to the table given below is worked into a hide on a calender at 170°C and subsequently pressed into a one mm thick sheet at 230°C and a pressure of 40 kg/cm<sup>2</sup>. The sheets thus obtained are subjected to an accelerated oxygen ageing at 140°C (air, normal pressure). The time which elapses until the first visually perceptible cracks arise is a measure of the antioxidant effect of the added compound.

EXAMPLE 3

60

65 TABLE 4

| Added Compound                          | Time until cracks form, in hours at 140°C |    |
|-----------------------------------------|-------------------------------------------|----|
|                                         | 5                                         | 25 |
| without additive                        |                                           |    |
| A. Commercially available antioxidants: |                                           |    |
| 2,6-Di-tert.butyl-4-methylphenol        |                                           |    |
|                                         | 5                                         | 25 |

|                                                             |     |
|-------------------------------------------------------------|-----|
| Methylene-bis-(3-methyl-4-hydroxy-<br>5-tert. butylbenzene) | 28  |
| B. Compounds according to the invention:                    |     |
| Formula (13)                                                | 850 |
| Formula (26)                                                | 620 |
| Formula (30)                                                | 400 |
| Formula (31)                                                | 320 |

#### EXAMPLE 4

In parallel experiments, freshly distilled olive oil is oxidized for 20 minutes at 140° C in a pure oxygen stream, both without additives and also with the addition of, in each case, 0.2 percent by weight of the compounds quoted in Table 5 below. Thereafter one g of the batch is dissolved in a mixture of 20 ml of carbon tetrachloride, 20 ml of chloroform and 20 ml of freshly distilled glacial acetic acid. The oxygen dissolved in the form of a gas is expelled by means of a strong stream of nitrogen, after which one ml of saturated potassium iodide solution is added. The mixture is then well stirred for five

minutes under a nitrogen atmosphere so as to result in a quantitative separation of iodine. After adding 100 ml of freshly distilled water and a little starch solution as the indicator, the mixture is immediately back-titrated with 0.002 N sodium thiosulphate solution until the blue color disappears.

Peroxide number (= milliequivalents of peroxidic oxygen)/kg = ml (sodium thiosulphate solution) · 2

TABLE 5

- Olive oil, without additive, freshly distilled
- Olive oil, without additive, oxidized for 20 minutes
- Olive oil with 0.2 % of the compound 13 (partially dissolved) (Example 1)
- Olive oil with 0.2 % of the compound 26 (Example 2)

### EXAMPLES

A mixture of 100 g of polyethylene powder (Microthene)

722, USI) and 0.2 g of one of the compounds mentioned in Table 6 is aged at 85°C for 16 hours in a circulating air oven. Thereafter the melt index is determined according to ASTM Specification D-1238-62-T. The melt index equals the amount of polyethylene, in grams, which has flowed in 10 minutes through a standard die, and represents a measure of

the degradation of the polymeric material. In a comparison experiment, the melt index of polyethylene samples without additives is determined.

TABLE 6

|    |                                                                                          | Melt index |
|----|------------------------------------------------------------------------------------------|------------|
| 10 | Polyethylene, without additive, not aged                                                 | 3.48       |
|    | Polyethylene, without additive, aged                                                     | 3.81       |
|    | Polyethylene with 0.2 part of the compound 13<br>(Example 1)                             | 3.56       |
| 15 | Polyethylene with 0.2 of the compound 26<br>(Example 2)                                  | 3.50       |
|    | Polyethylene with 0.2 part of 2,6-di-tert.butyl- 4-<br>methylphenol                      | 3.53       |
|    | Polyethylene with 0.2 part of methylene-bis-<br>(3-methyl-4-hydroxy-5-tert.butylbenzene) | 3.63       |

We claim:

### 1. A carboxylic acid amide of the formula



30 wherein M denotes a divalent bridge member of the series, —S—A—S— and —S—CH<sub>2</sub>—CH<sub>2</sub>—(O—CH<sub>2</sub>—CH<sub>2</sub>)<sub>p</sub>—S—, A denotes an alkylene containing one to 18 carbon atoms, p denotes an integer from one to three, R<sub>1</sub> denotes an alkyl group with one to eight carbon atoms and R<sub>2</sub> denotes hydrogen or an alkyl group with one to eight carbon atoms.

**2. A carboxylic acid amide according to claim 1, which corresponds to the formula**



wherein  $M_1'$  denotes a divalent bridge member  $—S—(CH_2)_q—S—$  or  $—S—CH_2—CH_2—O—CH_2—CH_2—S—$ ,  $q$  denotes an integer from one to six,  $n$  denotes an integer from one to 12,  $R_1$  denotes an alkyl group with one to eight carbon atoms,  $R_2$  denotes hydrogen or an alkyl group with 1 to eight carbon atoms and  $R_2'$  denotes hydrogen or an alkyl group containing one to four carbon atoms;  $R_2$  and  $R_2'$  cannot simultaneously be different from hydrogen.

3. A carboxylic acid amide according to claim 1 which corresponds to the formula



50 wherein  $M_1$  denotes a divalent bridge member  $—S—(CH_2)_q—S—$ ,  $q$  denotes an integer from one to six,  $n$  denotes an integer from one to 12,  $R_1$  denotes an alkyl group with one to eight carbon atoms and  $R_2$  denotes hydrogen or an alkyl group with one to eight carbon atoms.

55 4. A carboxylic acid amide according to claim 1, which corresponds to the formula



wherein  $M_1$  denotes a divalent bridge member  $—S—(CH_2)_q—S—$ ,  $q$  denotes an integer from one to six,  $m$  denotes an integer from one to four and  $R_3$  denotes a branched alkyl group containing up to four carbon atoms.

\* \* \* \*

UNITED STATES PATENT OFFICE  
CERTIFICATE OF CORRECTION

Patent No. 3,676,494

Dated July 11, 1972

Inventor(s) HANS RUDOLF BILAND ET AL

It is certified that error appears in the above-identified patent  
and that said Letters Patent are hereby corrected as shown below:

Column 1, after "Assignee:" delete "Ciba Limited" and  
substitute --- CIBA-GEIGY AG ---.

Signed and sealed this 16th day of April 1974.

(SEAL)

Attest:

EDWARD M.FLETCHER, JR.  
Attesting Officer

C. MARSHALL DANN  
Commissioner of Patents

aaa